

Aug. 26, 1969

HITOSHI IMAMIYA ET AL

3,463,655

PRESSURE-SENSITIVE COPYING PAPER

Filed April 5, 1967



INVENTORS

HITOSHI IMAMIYA  
SHIZUO KATAYAMA  
HIROHARU MATSUKAWA  
TERUO KOBAYASHI  
SADAO ISHIGE

BY *Aughine, Rothwell, Nixon, Ekin & Maguire*

ATTORNEYS

1

3,463,655

PRESSURE-SENSITIVE COPYING PAPER  
 Hitoshi Imamiya, Shizuo Katayama, and Hiroharu Matsukawa, Fujimiya-shi, and Teruo Kobayashi and Sadao Ishige, Ashigara-Kamigun, Japan, assignors to Fuji Shashin Film Kabushiki Kaisha, Ashigara-Kamigun, Kanagawa, Japan

Filed Apr. 5, 1967, Ser. No. 628,754  
 Claims priority, application Japan, Apr. 9, 1966,

41/22,196

Int. Cl. B41m 5/16, 5/14

U.S. Cl. 117—36.2

4 Claims

## ABSTRACT OF THE DISCLOSURE

A pressure-sensitive copying paper containing as a color former a coumarin compound of the following general formula:



Suitable coumarin compounds of the above type are 4 - methyl - N,N - dimethyl - aminocoumarin, 4 - methyl - N,N - diethyl - aminocoumarin, 4 - propyl - 7 - N - ethyl - N - benzyl - aminocoumarin, 4 - phenyl - 7 - N,N - diethyl - aminocoumarin, 4 - (4' - methoxyphenyl) - 7 - N,N - dimethyl - aminocoumarin and 4 - (3' - methylphenyl) - 7 - N,N - diethyl - aminocoumarin. The coumarin may be used with or without leuco color forming compounds conventionally used in reaction-type pressure-sensitive, copying papers. The copy obtained with the new copying paper can be efficiently reproduced by diazo and electrophotographic printing or copying systems.

## BACKGROUND OF THE INVENTION

### Field of the invention

This invention relates to a pressure-sensitive copying paper using a coumarin compound as a color former and it is concerned with pressure-sensitive copying paper which provides colored marks which can be reproduced, if desired, by an electrophotographic copying system or a diazo-type printing system.

Commercial pressure-sensitive copying papers utilize the phenomenon that when a colorless electron-donor, organic compound is adsorbed on an electron-acceptor adsorbent, both of the colorless materials are converted into a colored material. In such pressure-sensitive copying systems, a paper is coated with a dispersion of nonvolatile, fine liquid droplets containing a colorless electron-donor, organic compound encapsulated in a microcapsule which is capable of being ruptured by local pressure, e.g., by means of a pencil, stylus, ball-point pen and typewriter. A second paper is coated with a film of a finely divided adsorbent in a binder, and they are closely superimposed on each other and pressed locally. In this way, color is formed only in the pressed region.

### Discussion of the prior art

When the most commonly used color former for pressure-sensitive copying papers, for example, a leuco com-

2

pound, such as, Leuco Methylene Blue or Crystal Violet Lactone, is adsorbed on a clay, such as, kaolin or bentonite, which are electron-acceptor adsorbents, the absorption wave length of the thus colored marks appears within a range of 550 to 700 millimicrons. Such colored marks, therefore, are hardly able to be copied on diazo copying paper, when submitted to a diazo copying procedure, and also lacks the ability to be efficiently copied by electrophotography.

Thus, the principal object of the invention is to overcome the foregoing disadvantages of known pressure-sensitive copying papers.

## SUMMARY OF THE INVENTION

The present invention is based upon our discovery that the use of a compound represented by the following general formula:



in which R<sub>1</sub> and R<sub>2</sub> each is a member selected from the group consisting of a lower alkyl group and an aralkyl group, and R<sub>3</sub> is a member selected from the group consisting of a lower alkyl group and an aryl group, as a color former in a color forming reaction with an electron-acceptor adsorbent, such as, clays, result in the formation of colored marks having an absorption wave length substantially within a range of 380 to 400 millimicrons and colored light yellow. This is an absorption range most suitable for the light-sensitive zone of the commercial diazo copying paper.

## BRIEF DESCRIPTION OF THE DRAWING

The invention is illustrated in the accompanying drawing which sets forth spectral absorption curves for markings or images formed with the present copying materials.

## DETAILED DESCRIPTION OF THE INVENTION

In the drawing, there are shown spectral absorption curves for markings obtained with a clay paper and a conventional paper that have been immersed in a benzene solution of 4-methyl-7-diethylaminocoumarin, one of the compounds of our invention, and then dried. Curve 1 shows the absorption spectrum of marks obtained by applying the coating on the clay paper and curve 2 is the absorption spectrum for markings obtained by applying the coating on the conventional paper. As is evident from the curves, use of the coumarin compounds of this invention gives markings having a maximum absorption near 385 millimicrons. The colored marks obtained by using the coumarin as a color former, with or without the foregoing leuco compounds, for pressure-sensitive copying papers and subjecting such papers to color forming reactions with clay according to the foregoing procedure, can be readily copied by diazo-type and electrophotographic reproduction procedures. In the case of using only the color forming compound of our invention, however, the color formed on a clay paper is light yellow and is not a clear color. However, this disadvantage is readily overcome by the joint use of the conventional leuco compound described above.

The following compounds are illustrative of the color former compound used in the invention although the in-

vention shall not be limited to them. Each structural formula thereof is represented by substituents  $R_1$ ,  $R_2$  and  $R_3$  of the foregoing general formula.

TABLE 1

| Color<br>Former No. | $R_1$                   | $R_2$                                                                                             | $R_3$                                                                             | Compound                                           |
|---------------------|-------------------------|---------------------------------------------------------------------------------------------------|-----------------------------------------------------------------------------------|----------------------------------------------------|
| I                   | $-\text{CH}_3$          | $-\text{CH}_3$                                                                                    | $-\text{CH}_3$                                                                    | 4-methyl-7-N,N-dimethyl-aminocoumarin.             |
| II                  | $-\text{C}_2\text{H}_5$ | $-\text{C}_2\text{H}_5$                                                                           | $-\text{CH}_3$                                                                    | 4-methyl-7-N,N-diethyl-aminocoumarin.              |
| III                 | $-\text{C}_2\text{H}_5$ | $-\text{CH}_2-$  | $-\text{C}_2\text{H}_5$                                                           | 4-propyl-7-N-ethyl-N-benzyl-aminocoumarin.         |
| IV                  | $-\text{C}_4\text{H}_9$ | $-\text{C}_4\text{H}_9$                                                                           |  | 4-phenyl-7-N,N-dibutyl-aminocoumarin.              |
| V                   | $-\text{CH}_3$          | $-\text{CH}_3$                                                                                    |  | 4-(4'-methoxyphenyl)-7-N,N-dimethyl-aminocoumarin. |
| VI                  | $-\text{CH}_3$          | $-\text{CH}_3$                                                                                    |  | 4-(2'-chlorophenyl)-7-N,N-dimethyl-aminocoumarin.  |
| VII                 | $-\text{C}_2\text{H}_5$ | $-\text{C}_2\text{H}_5$                                                                           |  | 4-(3'-methylphenyl)-7-N,N-diethyl-aminocoumarin.   |

A pressure-sensitive copying paper using the coumarin compounds of the invention, as mentioned above, as a color former, may be prepared in the conventional manner. Preparation of oil-involving capsules, for example, may be carried out according to the coacervation process as disclosed in U.S. Patents 2,800,457 and 2,800,458.

The feature of the pressure-sensitive copying paper of the present invention consists in the use of the coumarin compound as a color former, whereby there are provided colored marks giving an absorption wave length suitable for diazo copying papers. The properties of the pressure-sensitive copying paper are influenced by the manner in which it is prepared. Therefore, as is well known in the art, various raw materials for pressure-sensitive copying papers may be utilized and the preparation of a coating solution and the preparation, application and drying of the coating compositions may be carried out by any conventionally used apparatus or plant.

#### PREFERRED EMBODIMENTS OF THE INVENTION

The following examples are given in order to illustrate the invention:

##### Example 1

3.5 parts by weight of 4-methyl-7-N,N-diethyl-aminocoumarin (Color Former No. II of Table 1) was dissolved in 97 parts by weight of a mixed oil of trichlorodiphenyl and kerosene in a proportion of 4:1 at 60-70° C. (This is simply called color former oil.) 1.0 kg. of gum arabic and 1.0 kg. of gelatin, treated with acid, were dissolved in 4 liters of water at 40° C. and mixed with 0.12 kg. of Turkey red oil as an emulsifier, in which 5.0 kg. of the color former oil was then dispersed with stirring until the size of the oil drops was from 3 to 6 microns. The so obtained emulsion was diluted with water at 40-50° C. to 90:1, and its pH was adjusted to from 4.0 to 4.2 by the addition of 10% acetic acid with stirring, thereby accumulating a colloid around the oil drops to form capsules. Continuing the stirring for about 20 minutes, the capsules were cooled from the outside by ice water and gelled or fixed. At 20° C., 1 liter of 37% formalin was added thereto to harden the fixed walls of the capsules.

Where it is desired to harden them further, an aqueous 15% caustic soda solution is added to adjust the pH to from 9 to 10 and the softening point is thus raised.

After 30 minutes, the capsule solution was heated with stirring for 20 minutes to 50° C. and applied to a suitable

support member in a predetermined coating amount by means of an air knife coating or roll coating, followed by drying, to obtain a pressure-sensitive copying paper.

When a colored mark formed on a clay paper by the use of the pressure-sensitive copying paper made by the foregoing procedure, was subjected to commercial diazo copying, a very sharp copied image was obtained.

Similarly, when subjected to electrophotographic copying, an excellent copied image was obtained which is quite different from the experience with the prior art.

The colored marking was resistant to radiation of sunlight, ultraviolet rays, arcs, and so on, over a long period of time. The coating surface was subjected to heat treatment at 150° C. for 10 hours and to radiation of ultraviolet rays for 1 hour, and then was used to form colored markings on a clay paper. The colored markings so produced were scarcely influenced by the pretreatment of the paper.

##### Example 2

This example is similar to Example 1 except that 3.5 parts by weight 4-methyl-7-N,N-diethyl-aminocoumarin (Color Former No. II of Table 1), 4.5 parts by weight of Crystal Violet Lactone and 3 parts by weight of Benzoyl Leuco Methylene Blue were dissolved in 89 parts by weight of a mixed oil of trichlorodiphenyl and kerosene in a mix ratio of 4:1 and 5.0 kg. of the resulting color former oil was used.

A colored mark produced on a clay paper by the resulting pressure-sensitive copying paper was in no way inferior to that of known pressure-sensitive copying papers, which are free of the color former of the present invention, with respect to the color tone, density and other properties. Further, the paper produced a copy capable of being copied by diazo-type paper in a diazo copier. The copy also produces a copy having better contrast, than in the prior art, when subjected to electrophotography.

There was no change in the color signal even after exposure to sunlight, ultraviolet rays or arcs for a long time. When the coating surface was subjected to heat treatment at 150° C. for 10 hours and to radiation of ultraviolet rays and then a copy was formed by reaction with a clay paper, the colored marks produced were satisfactory and gave better results, in particular, in terms of light resistance than copies produced from materials free of the compound of the invention. This is perhaps due to the fact that the compound acts as an absorbent of ultraviolet rays.

##### Example 3

A pressure-sensitive copying paper was prepared in a similar manner to Example 2 except that 4 parts by weight

of 4-methyl - 7 - N,N - dimethyl - aminocoumarin (Color Former No. I of Table 1) was used in place of the Color Former No. II. A colored mark formed on a clay paper by the resulting pressure-sensitive copying paper was a copy image capable of being reproduced by diazo copying paper or electrophotography and otherwise performed satisfactorily as in the case of the materials of Example 2.

## Example 4

A pressure-sensitive copying paper was prepared in a similar manner to Example 2, except that 3.5 parts by weight of 4-propyl-7-N-ethyl-N-benzyl-aminocoumarin (Color Former No. III) or 3.2 parts by weight of 4-phenyl-7-N,N-dibutyl-aminocoumarin (Color Former No. IV) or 3.0 parts by weight of 4-(4'-methoxyphenyl)-7-N,N-dimethyl-aminocoumarin (Color Former No. V) or 3.0 parts by weight of 4-(2'-chlorophenyl)-7-N,N-dimethyl-aminocoumarin (Color Former No. VI) or 3.0 parts by weight of 4-(3'-methylphenyl)-7-N,N-diethyl-aminocoumarin (Color Former No. VII) was used in place of the Color Former No. II of Table 1. Although some of the compounds were colored light yellow and the coating surfaces were colored light yellow in some of the resulting pressure-sensitive copying papers, colored markings formed on clay papers could be copied by diazo-type or electrophotographic copying procedures and increased the light resistance of the images where used together with a leuco compound color former.

What is claimed is:

1. A pressure sensitive copying transfer paper comprising a support and a transfer layer containing as a color former, at least one coumarin compound represented by the following general formula:



in which R<sub>1</sub> and R<sub>2</sub> each is a radical selected from the group consisting of lower alkyl and aralkyl radicals, and R<sub>3</sub> is a radical selected from the group consisting of lower alkyl and aryl radicals, said transfer layer being adapted to transfer said color former onto a second support which carries an electron-acceptor adsorbant thereon, whereupon a color forming reaction takes place between said color former and said electron acceptor adsorbant.

2. The pressure-sensitive copying paper as described in claim 1 wherein the coumarin compound is one selected from the group consisting of 4-methyl-N,N-dimethyl-aminocoumarin, 4-methyl-7-N,N-diethyl-aminocoumarin, 4 - propyl-7-N-ethyl-N-benzyl-aminocoumarin, 4 - phenyl-7-N,N-dibutyl - aminocoumarin, 4-(4'-methoxyphenyl)-7-

15 N,N - dimethyl - aminocoumarin, 4-(2'-chlorophenyl)-7-N,N-dimethyl-aminocoumarin and 4-(3'-methylphenyl)-7-N,N-diethyl-aminocoumarin.

3. The pressure-sensitive copying paper as described in claim 1 wherein said layer further contains a leuco compound which enters a color forming reaction with an electron-acceptor material.

4. The pressure-sensitive copying paper as described in claim 3 wherein said leuco compound is one selected from the group consisting of Crystal Violet Lactone and Leuco Methylene Blue.

## References Cited

## UNITED STATES PATENTS

|    |           |        |               |       |          |
|----|-----------|--------|---------------|-------|----------|
| 30 | 3,016,308 | 1/1962 | MacAulay      | ----- | 117-36.1 |
|    | 3,020,170 | 2/1962 | MacAulay      | ----- | 117-36.2 |
|    | 3,207,621 | 9/1965 | Newman et al. | ----- | 117-36.1 |

MURRAY KATZ, Primary Examiner

35

U.S. Cl. X.R.

117-156; 252-316